

[54] HEAT RESISTANT ALLOYS

|           |         |                      |        |
|-----------|---------|----------------------|--------|
| 3,279,915 | 10/1966 | Fujisawa et al. .... | 75/147 |
| 3,392,015 | 7/1968  | Badia ....           | 75/147 |
| 3,429,695 | 2/1969  | Nakamura et al. .... | 75/147 |
| 3,514,286 | 5/1970  | Unai et al. ....     | 75/147 |
| 3,666,451 | 5/1972  | Bewley ....          | 75/147 |
| 3,698,890 | 10/1972 | Bewley ....          | 75/147 |

[75] Inventor: Paul Zimmermann,  
Grimmlinghausen, Germany

[73] Assignee: Honsel-Werke AG, Meschede-Ruhr,  
Germany

[22] Filed: June 7, 1972

[21] Appl. No.: 260,556

Primary Examiner—W. Stallard  
Attorney, Agent, or Firm—Spencer & Kaye

[30] Foreign Application Priority Data

June 14, 1971 Germany ..... 2129352

[52] U.S. Cl. .... 75/147, 148/3, 148/159

[51] Int. Cl. .... C22c 21/04, C22f 1/04, F02f 1/24

[58] Field of Search ..... 75/147; 148/3, 159;  
29/183

[56] References Cited

UNITED STATES PATENTS

2,186,394 1/1940 Spitaler ..... 75/147

[57]

ABSTRACT

An aluminum-magnesium-silicon alloy with the customary additions for the production of parts such as cylinder heads, for resisting high alternating stressing and also high thermal stressing, wherein the improvement comprises the presence of grain-refined  $Mg_2Si$  and a component for reducing the solubility of hydrogen.

9 Claims, 3 Drawing Figures



○ = MEASURED VALUES FROM TABLE 8  
● = AVERAGE VALUES FROM TABLE 8  
⊗ = AVERAGE VALUE FROM TABLE 7  
OTHER ALLOYING COMPONENTS

TABLE 8

|                  |                  |
|------------------|------------------|
| 0.98 - 1.00 % Si | 0.94 - 0.99 % Si |
| 0.89 - 0.92 % Mn | 0.36 % Mn        |
| 0.50 - 0.55 % Cu | 0.52 - 0.55 % Cu |
| 0.15 % Ti        | n.b. % Ti        |
| 0.33 - 0.45 % Fe | 0.43 - 0.45 % Fe |
| 0.004% Be        | n.b. % Be        |
| BALANCE Al       | BALANCE Al       |

TABLE 7

n.b. = NOT DETERMINED

FIG.1



○ = MEASURED VALUES FROM TABLE 8

● = AVERAGE VALUES FROM TABLE 8

◎ = AVERAGE VALUE FROM TABLE 7

OTHER ALLOYING COMPONENTS

TABLE 8

0.98 - 1.00 % Si  
0.89 - 0.92 % Mn  
0.50 - 0.55 % Cu  
0.15 % Ti  
0.33 - 0.45 % Fe  
0.004% Be  
BALANCE Al

TABLE 7

0.94 - 0.99 % Si  
0.36 % Mn  
0.52 - 0.55 % Cu  
n. b. % Ti  
0.43 - 0.45 % Fe  
n. b. % Be  
BALANCE Al

n. b. = NOT DETERMINED

PATENTED FEB 25 1975

3,868,250

SHEET 2 OF 2

FIG. 2



FIG. 3

## HEAT RESISTANT ALLOYS

## BACKGROUND OF THE INVENTION

The present invention relates to AlMgSi alloys with the customary additives and to a material thereof for the production of parts resisting highly cyclic loads and of high thermal stresses, to the use of such alloys and of materials thereof for heat-resistant parts, and to components made of these materials.

As a consequence of the higher requirements placed on a wide variety of different designs at the present time, metallic materials must withstand higher stresses as well. These higher stresses of materials occur at lower and higher temperatures. Changes in the composition of alloys have become, therefore, necessary. Some alloys, among these the heat-resistant aluminum-magnesium-silicon alloys, represent an exception. They have been cast for decades in the same composition.

Investigations for an improvement of aluminum-magnesium-silicon alloys were made almost three decades ago. These experiments related particularly to the improvement of the age-hardenability of alloys with 3% magnesium and 0.8% silicon. Through an addition of cerium the magnesium-silicide could be grain-refined. With further additions of 0.8% zinc and 0.8% manganese alloyed together with cerium, a further improvement was obtained which was, however, not so distinct as that effected by the addition of cerium. This alloy has not been used.

Later, others carried out extensive experiments with extruded aluminum-magnesium-silicon alloys in order to make the quasibinary, the ternary and the below-eutectic compositions usable for heat-resistant purposes. These experiments were not continued although also here the hot-strength inherent in aluminum-magnesium alloys was noted and could be improved by other alloying constituents.

These and other numerous experiments have led to the use of aluminum-magnesium-silicon alloys, containing: 2-5.5% magnesium; 0-1.5% silicon; 0-0.6% manganese; 0-0.20% titanium, balance aluminum. For heat-resistant purposes, mainly for use as cylinder head material, an aluminum base alloy with the almost equal composition, used by all foundries, of 4.8-5.5% magnesium, 0.8-1.2% silicon, 0.4-0.6% copper, the above manganese content range, balance aluminum, was normally delivered. As per agreement with the purchaser, small quantities of beryllium were sometimes added to these alloys for inhibiting oxidation.

The ranges for the magnesium and silicon contents of these alloys permit a wide variation in the quantity of magnesium silicide which can be formed. Furthermore, magnesium not combined with silicon is found in the alloys. This is shown in Table 1.

Table 1

| Total Mg % | Combined and Uncombined Magnesium Si-content in % | Magnesium not combined with Si in % | Approximate solidus in the system AlMg in °C |
|------------|---------------------------------------------------|-------------------------------------|----------------------------------------------|
| 4          | 0.6                                               | 2.97                                | 604                                          |
| 4          | 1.0                                               | 2.27                                | 617                                          |
| 4          | 1.5                                               | 1.41                                | 635                                          |
| 4.8        | 0.6                                               | 3.77                                | 592                                          |
| 4.8        | 1.0                                               | 3.07                                | 603                                          |
| 4.8        | 1.5                                               | 2.21                                | 615                                          |

Table 1-Continued

| Total Mg % | Combined and Uncombined Magnesium Si-content in % | Magnesium not combined with Si in % | Approximate solidus in the system AlMg in °C |
|------------|---------------------------------------------------|-------------------------------------|----------------------------------------------|
| 5.5        | 0.6                                               | 4.47                                | 580                                          |
| 5.5        | 1.0                                               | 3.77                                | 592                                          |
| 5.5        | 1.5                                               | 2.91                                | 605                                          |
| 7.0        | 0.6                                               | 5.97                                | 557                                          |
| 7.0        | 1.0                                               | 5.27                                | 568                                          |
| 7.0        | 1.5                                               | 4.41                                | 581                                          |

## SUMMARY OF THE INVENTION

An object of the invention is to provide an aluminum-magnesium-silicon alloy especially resistant to thermal fatigue.

20 This as well as other objects which will become apparent in the discussion that follows are achieved, according to the present invention, by an aluminum-magnesium-silicon alloy having grain-refined  $Mg_2Si$  and a component for reducing the solubility of hydrogen.

## GENERAL ASPECTS OF THE INVENTION

Toward the end of improving the alloys mentioned in the above BACKGROUND OF THE INVENTION, numerous experiments have been made. These experiments 30 were based on the working hypothesis that aluminum-magnesium-silicon alloys for withstanding high stresses, in particular for withstanding alternating thermal stresses, must possess magnesium and silicon contents equilibrated to each other, and that the free magnesium content uncombined with silicon must not exceed beyond limits the solid solubility of magnesium in aluminum at room temperature.

Especially the use of the alloys mentioned in the BACKGROUND OF THE INVENTION for cylinder 40 heads gave rise to the recognition that cracking caused by the temperatures prevailing in the combustion chamber occurs earlier at higher magnesium contents. A reduction of the magnesium content to lower concentrations should also be of advantage for increasing 45 the solidus point of the alloys.

Besides establishing the influence of magnesium content, numerous investigations were made for establishing the influences of various other alloying constituents. Prior to casting, the melts were extensively degassed and only such elements were added, the addition of which was known not to increase the solubility of hydrogen. Furthermore, the solidus points in the aluminum-magnesium-silicon system were not to be decreased considerably, and in addition the grain refinement of the structure was to be improved. Combined with the component for reducing the solubility of hydrogen, it is important for obtaining the best grain-refinement in the  $Mg_2Si$ , i.e., for maximizing the 50 fineness of the  $Mg_2Si$  grains, that an extra measure be taken to assure no hydrogen evolution occurs during the time that the alloys are cooling from the molten condition to solidification to disturb the formation of a fine microstructure. Such evolution is prevented by the intensive degassing at the time of casting. An equilibrium condition, under which no hydrogen evolution occurs, is obtained right at the time of solidification. This equilibrium condition corresponds to a certain maximum 55

amount of hydrogen dissolved in the melt at the time of casting.

It was found that, when casting aluminum-magnesium-silicon alloys in permanent molds having a temperature of 300° C, a finer distribution of Mg<sub>2</sub>Si is obtained, the smaller the magnesium content of the alloy is that is not combined with silicon, and that through an increased manganese content in the absence of cerium and zinc, a still finer Mg<sub>2</sub>Si is obtained which at low magnesium content is recognized only at a very high magnification microscopically as a very fine precipitate. The influence of manganese on mechanical properties is consequently outstanding at room temperature and elevated temperatures as shown in Table 2. The tensile test specimens of Table 2 were subjected to a stabilizing annealing before testing. The stabilizing annealing causes a major separating of solid solution crystals into separate phases and thus represents a softening anneal. Growth changes are prevented by this. Decisive is a major stabilizing against the effects of later heating. When used, the material experiences no further changes. The stabilizing annealing effects an annealing, a stabilizing, and a stress relieving.

In the Tables, the following symbols are used:

$\sigma_{0.2}$  = yield strength

$\sigma_B$  = breaking strength

$\delta_s$  = elongation

HB = Brinell hardness.

The specimens for obtaining the data specified in Table 2 had a length of 22 cm and an original diameter of 2.2 cm over the whole gage length. They were made by chill casting at casting temperatures of approximately 720° to 750° C. The diameter over the gage length was obtained by turning on a lathe from the as cast diameter of 2.2 cm to 1.6 cm. The castings had a riser over their entire length. The mold, open at the top, was filled from one side through a gate. The chill 10 was horizontal and had a temperature of 300° C.

The addition of manganese should not exceed the maximum solid solubility in the aluminum-manganese system, but it should also not be lower than 0.6%.

The grain refining of the structure of Mg<sub>2</sub>Si through 15 the action of manganese has nothing in common with the forming of pointed, needle-shaped iron aluminides by manganese in aluminum-silicon-alloys with low magnesium-contents from 0 up to approximately 0.6%. It is true that in Al-Mg-Si alloys with Fe-contents of 20 1.25%, Mg<sub>2</sub>Si can be refined by higher manganese-contents, but a forming of the iron aluminide into a multi-substance compound cannot occur as is the case with aluminum-silicon alloys. These alloys have low elongation and strength properties, as shown in Table 25 3.

The pointed iron aluminide structure found in the aluminum-magnesium-silicon alloys of Table 3 is not prevented in the ternary aluminum-silicon-magnesium

Table 2

| Charge No. | Analysis in % |      |      |       | Tests at 20°C                         |                                   |                 | Tests at 300°C            |                                       |                                   | Tests at 400°C       |                                       |                                   |                 |
|------------|---------------|------|------|-------|---------------------------------------|-----------------------------------|-----------------|---------------------------|---------------------------------------|-----------------------------------|----------------------|---------------------------------------|-----------------------------------|-----------------|
|            | Mg            | Si   | Mn   | Fe    | kp*/mm <sup>2</sup><br>$\sigma_{0.2}$ | kp*/mm <sup>2</sup><br>$\sigma_B$ | %<br>$\delta_s$ | kp*/mm <sup>2</sup><br>HB | kp*/mm <sup>2</sup><br>$\sigma_{0.2}$ | kp*/mm <sup>2</sup><br>$\sigma_B$ | %<br>$\delta_s$      | kp*/mm <sup>2</sup><br>$\sigma_{0.2}$ | kp*/mm <sup>2</sup><br>$\sigma_B$ | %<br>$\delta_s$ |
| 850        | 3.6           | 1.04 | 0.22 | 0.31  | 7.6<br>7.9                            | 17.9<br>16.3                      | 7.4<br>4.8      | 55<br>53<br>5.5           | 6.1<br>6.1<br>8.4                     | 8.4<br>8.9<br>44.4                | 78.0<br>63.8<br>44.4 | 2.8<br>2.8<br>4.7                     | 4.3<br>4.7<br>84.0                | 46.0<br>84.0    |
|            |               |      | Avg. | value | 7.7                                   | 17.1                              | 6.1             | 54                        | 5.9                                   | 8.6                               | 62.1                 | 2.8                                   | 4.5                               | 65.0            |
| 856        | 3.2           | 0.93 | 0.98 | 0.3   | 6.9<br>7.1                            | 20.8<br>20.7                      | 14.3<br>14.9    | 57<br>55<br>5.6           | 6.4<br>4.9<br>9.0                     | 9.7<br>9.1<br>35.4                | 42.4<br>36.4<br>35.4 | 4.1                                   | 6.2                               | 78.0            |
|            |               |      | Avg. | value | 7.0                                   | 20.7                              | 14.6            | 56                        | 5.6                                   | 9.3                               | 38.1                 | 4.1                                   | 6.2                               | 78.0            |
| 852        | 5.2           | 1.02 | 0.93 | 0.3   | 10.3<br>10.0                          | 22.2<br>21.0                      | 7.1<br>6.0      | 64<br>64<br>7.6           | 8.2<br>6.4<br>10.5                    | 11.7<br>11.0<br>25.4              | 30.6<br>25.8<br>25.4 | 4.1                                   | 6.2                               | 84.0            |
|            |               |      | Avg. | value | 10.1                                  | 21.6                              | 6.5             | 64                        | 7.4                                   | 11.1                              | 27.3                 | 4.1                                   | 6.2                               | 84.0            |
| 858        | 5.4           | 1.02 | 0.93 | 0.38  | 12.9<br>12.1                          | 26.5<br>26.9                      | 8.5<br>10.8     | 69<br>72<br>6.2           | 9.7<br>10.7<br>11.0                   | 13.6<br>13.4<br>41.2              | 71.4<br>33.2<br>41.2 | 5.3<br>5.3<br>7.8                     | 7.8<br>7.8<br>83.4                |                 |
|            |               |      | Avg. | value | 12.5                                  | 26.7                              | 9.6             | 70                        | 8.9                                   | 12.7                              | 48.6                 | 5.3                                   | 7.8                               | 83.4            |
| 854        | 6.5           | 1.10 | 0.22 | 0.23  | 12.9<br>13.1                          | 23.2<br>23.5                      | 5.1<br>5.3      | 72<br>72<br>9.9           | 8.7<br>10.1<br>12.4                   | 14.1<br>14.7<br>18.0              | 4.1                  | 6.7                                   | 85.2                              |                 |
|            |               |      | Avg. | value | 13.0                                  | 23.3                              | 5.2             | 72                        | 9.6                                   | 13.8                              | 21.8                 | 4.1                                   | 6.7                               | 85.2            |
| 860        | 6.6           | 1.17 | 0.9  | 0.36  | 13.7<br>13.7                          | 23.22<br>24.2                     | 4.0<br>4.9      | 74<br>76<br>9.4           | 9.9<br>9.2<br>13.6                    | 13.9<br>14.6<br>18.6              | 24.8<br>18.0<br>18.6 | 5.1                                   | 7.9                               | 97.0            |
|            |               |      | Avg. | value | 13.7                                  | 23.5                              | 4.4             | 75                        | 9.5                                   | 14.0                              | 20.5                 | 5.1                                   | 7.9                               | 97.0            |

\* p = ponds

Further concerning Table 2 and subsequent Tables herein, the test bars had a gage diameter of 16 mm and a gage length of 80 mm, i.e., 5-fold diameter. The elongation measured in the tensile testing machine during the tension test until break of the test bar is the elongation  $\delta_s$  stated in per cent of the original length of 80 mm.

alloys with approximately 13% silicon and 6% magnesium by an increased addition of manganese. Such experiments show in regard to the strength properties also no outstanding technical progress for a combination with manganese; they show also that in an application of manganese in the presence of large quantities of silicon and larger quantities of magnesium the effect of

manganese is not comparable to that in aluminum-silicon alloys with up to 0.6% magnesium or without magnesium. See Table 4.

shows the improvement of strength properties caused by manganese in alloys lying approximately in the melting valley between the ternary, magnesium-rich and

Table 3

| Charge No. | Analysis in % |      |      |      | Tests at 20°C                         |                                   |                 | Tests at 300°C                        |                                   |                 | Tests at 400°C                        |                                   |                 |      |
|------------|---------------|------|------|------|---------------------------------------|-----------------------------------|-----------------|---------------------------------------|-----------------------------------|-----------------|---------------------------------------|-----------------------------------|-----------------|------|
|            | Mg            | Si   | Mn   | Fe   | kp*/mm <sup>2</sup><br>$\sigma_{0.2}$ | kp*/mm <sup>2</sup><br>$\sigma_B$ | %<br>$\delta_s$ | kp*/mm <sup>2</sup><br>$\sigma_{0.2}$ | kp*/mm <sup>2</sup><br>$\sigma_B$ | %<br>$\delta_s$ | kp*/mm <sup>2</sup><br>$\sigma_{0.2}$ | kp*/mm <sup>2</sup><br>$\sigma_B$ | %<br>$\delta_s$ |      |
| 851        | 3.85          | 1.35 | 0.25 | 1.25 | 8.8                                   | 16.1                              | 2.8             | 57                                    | 5.3                               | 9.5             | 41.8                                  | 3.1                               | 4.8             | 79.0 |
|            |               |      |      |      | 8.9                                   | 18.8                              | 4.3             | 58                                    | 5.3                               | 8.9             | 47.2                                  | 2.8                               | 5.2             | 81.0 |
| Avg. value |               |      |      | 8.8  | 17.4                                  | 3.6                               | 57              | 5.3                                   | 9.2                               | 44.5            | 2.9                                   | 5.0                               | 80.0            |      |
| 857        | 3.8           | 1.10 | 0.9  | 1.25 | 9.4                                   | 17.1                              | 3.0             | 64                                    | 6.3                               | 10.7            | 12.2                                  | 3.6                               | 6.5             | 65.0 |
|            |               |      |      |      | 9.3                                   | 15.4                              | 2.1             | 62                                    | 4.8                               | 9.9             | 8.6                                   |                                   |                 |      |
| Avg. value |               |      |      | 9.3  | 16.2                                  | 2.5                               | 63              | 5.5                                   | 10.3                              | 10.4            | 3.6                                   | 6.5                               | 65.0            |      |
| 853        | 5.3           | 1.05 | 0.22 | 1.14 | 10.8                                  | 22.7                              | 4.8             | 71                                    | 8.4                               | 12.6            | 42.0                                  | 4.1                               | 6.7             | 98.2 |
|            |               |      |      |      | 10.5                                  | 22.5                              | 5.0             | 71                                    | 8.3                               | 11.6            | 33.8                                  |                                   |                 |      |
| Avg. value |               |      |      | 10.6 | 22.6                                  | 4.9                               | 71              | 8.3                                   | 12.1                              | 37.9            | 4.1                                   | 6.7                               | 98.2            |      |
| 859        | 5.5           | 1.14 | 0.82 | 1.00 | 10.3                                  | 18.5                              | 3.1             | 67                                    | 9.4                               | 13.1            | 7.8                                   | 4.2                               | 7.2             | 73.4 |
|            |               |      |      |      | 10.6                                  | 18.5                              | 2.9             | 72                                    | 7.6                               | 11.6            | 8.8                                   |                                   |                 |      |
| Avg. value |               |      |      | 10.4 | 18.5                                  | 3.0                               | 69              | 8.5                                   | 12.3                              | 7.3             | 4.2                                   | 7.2                               | 73.4            |      |
| 855        | 6.85          | 0.92 | 0.22 | 1.12 | 12.4                                  | 19.2                              | 2.4             | 76                                    | 9.4                               | 14.2            | 12.8                                  | 3.6                               | 6.2             | 64.6 |
|            |               |      |      |      | 12.4                                  | 22.8                              | 4.5             | 76                                    | 9.4                               | 13.8            | 17.0                                  |                                   |                 |      |
| Avg. value |               |      |      | 12.4 | 21.5                                  | 3.4                               | 76              | 9.4                                   | 14.0                              | 14.9            | 3.6                                   | 6.2                               | 64.6            |      |
| 861        | 7.0           | 1.06 | 0.87 | 1.20 | 14.1                                  | 18.8                              | 1.8             | 84                                    | 9.2                               | 14.7            | 4.2                                   | 4.1                               | 7.9             | 83.2 |
|            |               |      |      |      | 13.9                                  | 17.8                              | 1.3             | 90                                    | 9.2                               | 14.5            | 3.2                                   |                                   |                 |      |
| Avg. value |               |      |      | 14.0 | 18.3                                  | 1.5                               | 87              | 9.2                                   | 14.2                              | 4.9             | 4.1                                   | 7.9                               | 83.2            |      |

\* p = ponds

Table 4

| Charge No. | Analysis in % |       |      |      | Tests at 20°C                         |                                   |                 | Tests at 300°C                        |                                   |                 | Tests at 400°C                        |                                   |                 |      |
|------------|---------------|-------|------|------|---------------------------------------|-----------------------------------|-----------------|---------------------------------------|-----------------------------------|-----------------|---------------------------------------|-----------------------------------|-----------------|------|
|            | Mg            | Si    | Mn   | Fe   | kp*/mm <sup>2</sup><br>$\sigma_{0.2}$ | kp*/mm <sup>2</sup><br>$\sigma_B$ | %<br>$\delta_s$ | kp*/mm <sup>2</sup><br>$\sigma_{0.2}$ | kp*/mm <sup>2</sup><br>$\sigma_B$ | %<br>$\delta_s$ | kp*/mm <sup>2</sup><br>$\sigma_{0.2}$ | kp*/mm <sup>2</sup><br>$\sigma_B$ | %<br>$\delta_s$ |      |
| 888        | 6.0           | 13.57 | 0.21 | 0.29 | 9.6                                   | 16.9                              | 3.0             | 60                                    | 3.8                               | 7.6             | 11.6                                  | 2.4                               | 5.0             | 20.0 |
|            |               |       |      |      | 9.5                                   | 17.0                              | 2.8             | 58                                    |                                   |                 |                                       |                                   |                 |      |
| Avg. value |               |       |      | 9.5  | 16.9                                  | 2.9                               | 59              | 3.8                                   | 7.6                               | 11.6            | 2.4                                   | 5.0                               | 20.0            |      |
| 886        | 6.5           | 13.11 | 0.75 | 0.2  | 10.9                                  | 16.8                              | 2.0             | 66                                    | 5.6                               | 9.2             | 11.2                                  | 2.7                               | 4.2             | 20.0 |
|            |               |       |      |      | 10.5                                  | 17.2                              | 2.4             | 69                                    |                                   |                 |                                       |                                   |                 |      |
| Avg. value |               |       |      | 10.7 | 17.0                                  | 2.2                               | 67              | 5.6                                   | 9.2                               | 11.2            | 2.7                                   | 4.2                               | 20.0            |      |
| 889        | 5.25          | 12.95 | 0.22 | 1.3  | 10.9                                  | 12.2                              | 1.1             | 71                                    | 3.0                               | 8.8             | 1.8                                   | 2.9                               | 6.4             | 3.0  |
|            |               |       |      |      | 10.6                                  | 11.6                              | 0.8             | 69                                    |                                   |                 |                                       |                                   |                 |      |
| Avg. value |               |       |      | 10.7 | 11.9                                  | 0.9                               | 70              | 3.0                                   | 8.8                               | 1.8             | 2.9                                   | 64                                | 3.0             |      |
| 887        | 5.6           | 12.62 | 0.85 | 1.3  | 10.8                                  | 13.7                              | 1.4             | 71                                    | 6.3                               | 8.4             | 3.4                                   | 3.2                               | 5.8             | 7.2  |
|            |               |       |      |      | 10.5                                  | 14.8                              | 1.8             | 72                                    |                                   |                 |                                       |                                   |                 |      |
| Av. value  |               |       |      | 10.6 | 14.2                                  | 1.6                               | 71              | 6.3                                   | 8.4                               | 3.4             | 3.2                                   | 5.8                               | 7.2             |      |

\* p = ponds

After these investigations it was, therefore, astonishing that at very high magnesium-contents of approximately 9 - 10% and silicon-contents of approximately 3% at free magnesium-contents between 3 and 4% (magnesium not bound to silicon), also at higher iron-contents of 1.20%, iron-needles no longer occur, insofar as higher manganese-contents were added. However, in the presence of high quantities of iron, no considerable changes of strength properties have been caused. In the alloys with low iron-contents there is found by the manganese alloying, besides a strong refining of grain structure, a considerable increase of strength properties in connection therewith. Table 5

silicon-rich eutectics of the aluminum-silicon-magnesium system and preferably on the side rich on magnesium, and which have silicon-contents lower than those of the quasi-binary eutectic with 13% Mg<sub>2</sub>Si. Preferably silicon-contents between 2.5 and 4% and at most 11% magnesium should be alloyed in the presence of manganese.

The investigations were extended to alloys with silicon-contents of 2% and magnesium-contents of 4%. The strong refining of Mg<sub>2</sub>Si by manganese is obtained here as well.

With a Cu-content of 1% both in alloys poor on manganese and rich on manganese, Mg<sub>2</sub>Si is coarsened

again. It is most coarse in the alloys poor in manganese. Table 6 shows that a Cu-content increases strength properties, but that elongation properties are strongly decreased. The strength properties of Cu-free alloys with their higher magnesium-contents not bound to silicon, were not attained. At approximately 4% magnesium and 2% silicon, the alloy contains only 0.55% magnesium not bound to silicon. The machinability of castings from these alloys is worse.

Further results were obtained on investigation of the influence of nickel. Similarly to manganese, nickel contents of about 1% in aluminum show the lowest hydro-

gen solubility in the molten state. This composition was, therefore, also selected for alloying investigations. It was found that contrary to copper, a 1.5% nickel content gives a very fine magnesium-silicide and that the magnesium-silicide coarsening influence of copper is neutralized in the presence of nickel.

The investigation of tearing strength properties showed that the stabilized alloys, when the magnesium-content exceeds 4%, possess low elongation properties, 10 and that the aluminum-magnesium-silicon alloys must contain, in the presence of nickel and/or larger quantities than 0.2% copper, less than 4% magnesium.

Table 5

| Charge No. | Analysis in % |      |      |       | Tests at 20°C                         |                                   |                 | Tests at 300°C            |                                       |                                   | Tests at 400°C  |                                       |                                   |                 |
|------------|---------------|------|------|-------|---------------------------------------|-----------------------------------|-----------------|---------------------------|---------------------------------------|-----------------------------------|-----------------|---------------------------------------|-----------------------------------|-----------------|
|            | Mg            | Si   | Mn   | Fe    | kp*/mm <sup>2</sup><br>$\sigma_{0.2}$ | kp*/mm <sup>2</sup><br>$\sigma_B$ | %<br>$\delta_s$ | kp*/mm <sup>2</sup><br>HB | kp*/mm <sup>2</sup><br>$\sigma_{0.2}$ | kp*/mm <sup>2</sup><br>$\sigma_B$ | %<br>$\delta_s$ | kp*/mm <sup>2</sup><br>$\sigma_{0.2}$ | kp*/mm <sup>2</sup><br>$\sigma_B$ | %<br>$\delta_s$ |
| 871        | 9.7           | 3.1  | 0.28 | 0.2   | 14.9<br>14.9                          | 26.0<br>22.9                      | 3.4<br>2.1      | 92<br>92                  | 8.4<br>9.2                            | 12.8<br>13.6                      | 27.4<br>24.0    | 3.6                                   | 6.1                               | 74.8            |
|            |               |      | Avg. | value | 14.9                                  | 24.4                              | 2.7             | 92                        | 8.8                                   | 13.2                              | 25.7            | 3.6                                   | 6.1                               | 74.8            |
| 873        | 9.44          | 2.7  | 0.85 | 0.24  | 18.1<br>18.2                          | 27.5<br>27.2                      | 2.8<br>2.4      | 95<br>98                  | 12.2<br>11.2                          | 16.2<br>15.6                      | 35.4<br>13.6    | 4.8                                   | 8.5                               | 61.6            |
|            |               |      | Avg. | value | 18.1                                  | 27.3                              | 2.6             | 96                        | 11.7                                  | 15.9                              | 24.5            | 4.8                                   | 8.5                               | 61.6            |
| 947        | 8.6           | 3.3  | 0.32 | 0.30  | 11.9<br>12.1                          | 19.8<br>20.3                      | 1.8<br>2.0      | 80<br>78                  | 9.2<br>8.2                            | 13.9<br>11.7                      | 25.0<br>30.0    | —                                     | —                                 | —               |
|            |               |      | Avg. | value | 12.0                                  | 20.0                              | 1.9             | 79                        | 8.7                                   | 12.8                              | 27.5            | —                                     | —                                 | —               |
| 948        | 8.8           | 3.6  | 0.88 | 0.32  | 14.0<br>13.8                          | 25.3<br>25.4                      | 3.0<br>2.6      | 83<br>87                  | 9.2<br>9.6                            | 13.9<br>13.1                      | 19.6<br>23.6    | —                                     | —                                 | —               |
|            |               |      | Avg. | value | 13.9                                  | 25.3                              | 2.8             | 85                        | 9.4                                   | 13.5                              | 21.8            | —                                     | —                                 | —               |
| 872        | 9.25          | 3.1  | 0.30 | 1.20  | 16.0<br>15.6                          | 24.2<br>25.8                      | 3.5<br>3.1      | 101<br>91                 | 9.4<br>9.2                            | 14.3<br>14.3                      | 26.6<br>15.2    | 4.1                                   | 7.4                               | 83.6            |
|            |               |      | Avg. | value | 15.8                                  | 25.0                              | 3.3             | 96                        | 9.3                                   | 14.6                              | 19.7            | 4.1                                   | 7.4                               | 83.6            |
| 874        | 9.7           | 2.75 | 1.03 | 1.12  | 18.4<br>17.9                          | 23.5<br>24.8                      | 2.3<br>2.4      | 108<br>98                 | 13.5<br>8.1                           | 17.6<br>14.9                      | 5.2<br>6.6      | 5.1                                   | 8.1                               | 65.2            |
|            |               |      | Avg. | value | 18.1                                  | 24.1                              | 2.3             | 103                       | 10.8                                  | 16.2                              | 5.9             | 5.1                                   | 8.1                               | 65.2            |

\* p = ponds

Table 6

| Charge No. | Analysis in % |     |      |      |               | Tests at 20°C                         |                                   |                 | Tests at 300°C            |                                       |                                   |                 |
|------------|---------------|-----|------|------|---------------|---------------------------------------|-----------------------------------|-----------------|---------------------------|---------------------------------------|-----------------------------------|-----------------|
|            | Mg            | Si  | Mn   | Cu   | Fe            | kp*/mm <sup>2</sup><br>$\Sigma_{0.2}$ | kp*/mm <sup>2</sup><br>$\sigma_B$ | %<br>$\delta_s$ | kp*/mm <sup>2</sup><br>HB | kp*/mm <sup>2</sup><br>$\sigma_{0.2}$ | kp*/mm <sup>2</sup><br>$\sigma_B$ | %<br>$\delta_s$ |
| 940        | 3.95          | 2.0 | 0.24 | —    | 0.41          | 8.2<br>8.1                            | 17.8<br>17.6                      | 5.5<br>5.4      | 54<br>55                  | 4.4                                   | 7.7                               | 39.2            |
|            |               |     |      | —    | Avg.<br>value | 8.1                                   | 17.7                              | 5.4             | 54                        | 4.4                                   | 7.7                               | 39.2            |
| 944        | 4.2           | 1.9 | 1.00 | —    | 0.42          | 8.6<br>8.8                            | 18.6<br>18.6                      | 5.0<br>4.8      | 58<br>62                  | 4.9                                   | 7.5                               | 52.0            |
|            |               |     |      | —    | Avg.<br>value | 8.7                                   | 18.6                              | 4.9             | 60                        | 4.9                                   | 7.5                               | 52.0            |
| 942        | 4.35          | 2.2 | 0.23 | 1.04 | 0.43          | 10.3<br>10.3                          | 18.0<br>18.8                      | 2.8<br>3.3      | 66<br>64                  | 6.0                                   | 9.1                               | 35.4            |
|            |               |     |      | 1.04 | Avg.<br>value | 10.3                                  | 18.4                              | 3.0             | 65                        | 6.0                                   | 9.1                               | 35.4            |
| 946        | 4.00          | 1.8 | 0.9  | 1.0  | 0.24          | 11.0<br>10.6                          | 20.2<br>19.7                      | 3.9<br>3.0      | 69<br>67                  | 6.1                                   | 9.6                               | 39.6            |
|            |               |     |      | 1.0  | Avg.<br>value | 10.8                                  | 19.9                              | 3.4             | 68                        | 6.1                                   | 9.6                               | 39.6            |

\* p = ponds

## BRIEF DESCRIPTION OF THE DRAWINGS

FIG. 1 is a graph of alternating load number versus the percentage of free magnesium in an alloy.

FIG. 2 is a graph of the percentage of silicon in an alloy versus the percentage of magnesium and shows the field of free magnesium contents between 1 and 3%.

FIG. 3 is a cross section through a portion of an air-cooled cylinder head according to the invention.

## DESCRIPTION OF THE PREFERRED EMBODIMENTS

Preferred elements for reducing the solubility of hydrogen in the melt above 700° C are manganese and nickel.

The available results were applied to investigations of cylinder heads. The quality of service to be expected from an alloy used to make a cylinder head was measured in terms of "alternating load number," which is measured as follows.

On a heatable and coolable test stand, those portions of a cylinder head as are most endangered, being nearest to the combustion chamber, are heated for approximately 60 seconds from a temperature of 100° to 300° C and then cooled in 60 seconds to 100° C again. This effects a change of load. The test on the test stand is carried on until crack formation and then on until the crack has progressed through the wall where it is located. The number of load changes supported by the cylinder head until crack formation and until crack-through yields alternating load numbers, which serve as an indicator of the ability to resist thermal fatigue.

FIG. 1 shows among other things the alternating thermal stress tests of cylinder heads made of the customary alloy AlMg<sub>5</sub>Si<sub>1</sub>Cu0.5 per Table 7. The cylinder heads of Table 7 were taken from the normal production in a period extending over several months. There resulted an average alternating load number of 716 until crack formation and 769 until crack-through.

Cylinder heads cast from the material of the inven-

tion and showing a fine grain structure were likewise tested. FIG. 1 and Table 8 show the resulting alternating load numbers. It can be concluded from the investigations that with a silicon content comparable with the customary alloy, and with the customary addition of 0.5% Cu, alloys with high magnesium contents have a considerably shorter operating life even with an additional manganese-alloying. In comparison with the results for the customary alloy (see FIG. 1 and Tables 7 and 8), the alloys with higher manganese content show a distinct improvement. The graph in FIG. 1 shows an almost linear dependence between alternating load number and magnesium content and the possibility of a maximum improvement of 100% by the invention. The alloy used for cylinder head No. 3 in Table 8 and FIG. 1 possesses a free (i.e., not present in Mg<sub>2</sub>Si) magnesium-content of approximately 5.7%; the alloy of head No. 2 has a free magnesium-content of 3.77%; and the alloy of head No. 1 has a free magnesium-contents of only 2.85%. The alloys of heads No. 4 and No. 5 in Table 8 contain only about 0.9% free magnesium. The alloy of head No. 5 endures after the additional alloying of manganese considerably higher thermal loading. Comparison with the alloys of Table 7 shows the high thermal stress endurance obtained by the reduction of the free magnesium content. The free magnesium content of the alloys Nos. 4 and 5, being 0.9%, is very low. The machinability of these alloys was worse on a production line. The free magnesium contents should be more than 1%.

The alloys of the invention can also be used as wrought material, if the Si-content is at least 1%.

All investigations show that the free magnesium-contents of the aluminum-magnesium-silicon alloys for obtaining high endurance, specially against alternating thermal stresses, should be between 1 and 4.5, preferably at 3.0%, a decrease of free magnesium to less than 1% being possible only for castings that are machined with special tools adapted to the alloy. In the presence of more than 0.6% Mn the preferred 3% free magnesium can go up to about 4.5%.

Table 7

| Cylinder Head No. | Analysis in % |      |      |      |      | Alternating load No. |               |
|-------------------|---------------|------|------|------|------|----------------------|---------------|
|                   | Mg            | Si   | Mn   | Cu   | Fe   | Crack formation      | Crack-through |
| 1                 |               |      |      |      |      | n.b.                 | 709           |
| 2                 | 5.06          | 0.94 | 0.36 | 0.53 | 0.45 | 639                  | 670           |
| 3                 |               |      |      |      |      | 894                  | 960           |
| 4                 |               |      |      |      |      | 940                  | 1050          |
| 5                 |               |      |      |      |      | 450                  | 640           |
| 6                 | 5.19          | 0.99 | 0.36 | 0.52 | 0.44 | 775                  | 877           |
| 7                 |               |      |      |      |      | 707                  | 872           |
| 8                 |               |      |      |      |      | 574                  | 736           |
| 9                 |               |      |      |      |      | 640                  | 663           |
| 10                |               |      |      |      |      | n.b.                 | 760           |
| 11                |               |      |      |      |      | 830                  | 880           |
| 12                |               |      |      |      |      | n.b.                 | 650           |
| 13                | 5.16          | 0.95 | 0.36 | 0.55 | 0.43 | n.b.                 | 720           |
| 14                |               |      |      |      |      | n.b.                 | 660           |
| 15                |               |      |      |      |      | n.b.                 | 671           |
| 16                |               |      |      |      |      | n.b.                 | 800           |
| Average values    | 5.14          | 0.96 | 0.36 | 0.54 | 0.44 | ~716                 | ~769          |

n.b. = not precisely determinable

Table 8

| Cylinder Head No. | Analysis in % |      |      |      |      |      | Alternating load No. |                      |                      |
|-------------------|---------------|------|------|------|------|------|----------------------|----------------------|----------------------|
|                   | Mg            | Si   | Mn   | Cu   | Fe   | Ti   | Be                   | Crack formation      | Crack-through        |
| 1                 | 4.55          | 0.99 | 0.91 | 0.50 | 0.42 | 0.15 | 0.004                | 1450<br>1350         | 1600<br>1500         |
| 2                 | 5.5           | 1.00 | 0.92 | 0.50 | 0.32 | 0.15 | 0.004                | 800<br>1200          | 890<br>1224          |
| 3                 | 7.4           | 0.98 | 0.89 | 0.55 | 0.33 | 0.15 | 0.003                | n.b.<br>n.b.         | 168<br>335           |
| 4                 | 4.4           | 2.08 | 0.02 | 0.17 | 0.20 | 0.15 | 0.004                | 1040<br>930<br>n.b.  | 1160<br>1030<br>1100 |
| 5                 | 4.3           | 1.88 | 0.78 | 0.15 | 0.21 | 0.15 | 0.004                | 1380<br>1380<br>1360 | 1590<br>1420<br>1410 |

n.b. = not precisely determinable

During the further development of the alloys of the invention and of their applicability, it has been established by thermal alternating stress investigations that, within the range of the limits of the invention, alloys with the following alloying constituents have particularly favorable properties for enduring high-temperature alternating stresses and a particularly low cracking-tendency in engine operation:

|                                          |    |
|------------------------------------------|----|
| 3.5 - 7.0%                               | Mg |
| 0.8 - 2.5%                               | Si |
| 0.6 - 1.5%                               | Mn |
| 0.0 - 0.30%                              | Ti |
| 0.0 - 0.005%                             | Be |
| 0.0 - 0.05% other elements individually, |    |
| total however 0.15% maximum              |    |

Balance aluminum and customary contaminants, on the condition that only 1 to 3% magnesium unbound to silicon be contained in the alloy. A special importance is, in this instance, attributed to the proportioning of the manganese on which the increase of crack resistance in engine operation depends.

The proposed alloy selection results in particularly favorable mechanical properties. But all alloys, both those named first, and those selected now, yield especially improved mechanical properties and to the present time, the best crack resistance-against temperature changes, if the endangered or highly stressed areas of the cast body are subjected during the solidification to a cooling additional to the cooling received by other areas of the body. The behavior of alloys free of manganese shows in cylinder heads 30 to 50% of the durability achieved in cylinder heads made of alloys containing manganese.

FIG. 2 shows the range of preferred alloy compositions wherein only 1 to 3% free magnesium (not bound to silicon) is present.

Further illustrative of the invention are the following Examples:

#### EXAMPLE 1

Cylinder heads of the type illustrated by air-cooled

cylinder head 10 in FIG. 3 from an alloy poor in manganese, having the composition

25 0.3% Mn  
5.2% Mg  
1.0% Si  
0.004% Be  
balance Al and customary contaminants, were subjected to an alternating thermal stress investigation after cooling the permanent mold with about 700 cm<sup>3</sup> H<sub>2</sub>O in the area of the spherical cap 11. The cooling was carried out by flowing the water through a metal 30 mold core abutting against the spherical cap 11 and having cylinder inserts protruding into the inlet channel 12 and the outlet channel 13. The cooling effect provided by the cylinder inserts provides an additionally improved microstructure in the web 14, which is the most highly stressed portion of the head. The alternating load number was approximately 450 for the start of cracking of the web area between the inlet and outlet channels. Additionally in FIG. 3, axes 15, 16 and 17 are 35 axes of cylindrical symmetry for, respectively, the inlet channel 12, the spherical cap 11, and the outlet channel 13.

#### EXAMPLE 2

50 Cylinder heads of the same alloy as in Example 1 showed, after being cooled with 3.5 liters H<sub>2</sub>O in the same area, an alternating load number of 750.

#### EXAMPLE 3

Cylinder heads of the manganese rich alloy with the composition

55 0.9% Mn  
4.4% Mg  
1.0% Si  
0.004% Be  
balance Al and customary contaminants, were subjected, after cooling as in Example 2, to an alternating 60 thermal stress test and yielded an alternating load number of 1,550 to crackthrough.

## EXAMPLE 4

Under a more aggravated alternating thermal stress test consisting of a more rapid change of heating and cooling, cylinder heads according to Example 2 gave the reduced alternating load number of 650.

## EXAMPLE 5

Cylinder heads from alloys according to Example 3, tested according to Example 4, gave the alternating 10 load number of 1,200.

## EXAMPLE 6

Cylinder heads from the Mn rich alloy having the composition

0.85% Mn  
4.0% Mg  
1.2% Si  
0.004% Be

balance Al and customary contaminants, were, after cooling with 13 liters H<sub>2</sub>O according to Example 1, subjected to the alternating thermal stress test according to Example 4 and yielded an alternating load number of 2,220.

## EXAMPLE 7

Cylinder heads made from the alloy

0.85 % Mn  
4.7% Mg  
1.7% Si

balance as in Example 2, were tested on the test-bench for alternating thermal stresses according to Example 4 and endured 1,221 alternations of stress.

## EXAMPLE 8

Cylinder heads of the alloy according to Example 7 with only 0.3% Mn, tested on the test-bench for alternating thermal stresses as in Example 4, endured only 430 alternations of stress.

Table 9

| As per example | Alternating load number | Mechanical properties at 20°C                    |                                                     |                                   |      |
|----------------|-------------------------|--------------------------------------------------|-----------------------------------------------------|-----------------------------------|------|
|                |                         | Yield Stress kp/mm <sup>2</sup> σ <sub>0.2</sub> | Breaking Strength kp/mm <sup>2</sup> σ <sub>B</sub> | % Brinell Hardness δ <sub>5</sub> | HB   |
| 1              | 450                     | 10.8                                             | 19.8                                                | 2.7                               | 82.6 |
| 2              | 750                     | 12.6                                             | 21.2                                                | 3.7                               | 71.0 |
| 6              | 2220                    | 12.1                                             | 24.2                                                | 14.6                              | 68.0 |

\* p = ponds

The further development of the present invention is dedicated to showing a way of how the ability to endure high thermal stresses, particularly in cylinder heads cast from the aforementioned Al-Mg-Si alloys of the invention, can be considerably improved for obtaining a marked increase of engine operating life, alternating thermal stress endurance and considerably increased durability of sealing surfaces. This is done particularly by increased hardnesses of sealing surfaces, giving also an improvement of the compression chamber seal between cylinder block and cylinder head. So far, the sealing surface durability, which is connected with the Brinell hardness of the alloys, could not alone be considerably improved by concentration increases in the alloy, without at the same time reducing strongly the

ability to endure thermal fatigue in cylinder heads made from the alloys.

Especially for thermally highly stressed pieces, such as engine cylinder heads, it has so far been thought that the thermal treatment should consist only of a kind of stabilization annealing and that this cannot be improved, but only be deteriorated, by other treatments, particularly solution treatment alone or a solution treatment, and a subsequent age-hardening, which is customary for all other alloys. It is known that piston alloys for the prevention or reduction of increase in volume are homogenized at 500°C, with subsequent age-hardening, and annealed once more at temperatures of 250°C in the softening area, in order to attain complete growth resistance and freedom from stresses. However, the solution annealing treatment is not the rule for piston alloys, and it has been shown that also an exaggeratedly long annealing at 185°C from 16 to 40 hours, without solution treatment, is sufficient for stabilizing or prevention of growth. Beside that, temperatures of approximately 220°C have also been applied for annealing treatments alone.

The result of these thermal treatments is that alloying components come strongly out of solid solution. Thereby either maximum Brinell hardness properties with strongly decreased elongation properties or else very low Brinell hardness properties are obtained.

The intended further development of the invention involves subjecting the castings to either a solution treatment alone or to a solution treatment and subsequent age-hardening without exceeding the hardness maximum.

Investigations with this process have shown that a considerable improvement of all properties important for resistance to thermal fatigue, especially sealing surface hardness, is obtained, without disadvantage, with the applied thermal treatment. The results of such investigations are listed in Table 10 and become evident from the Examples of alternating thermal stressing of cylinder heads. Shown are the Brinell hardness properties and in individual cases strength properties in the border of the spherical cap of the cylinder heads. It was found that either a homogenizing or solution treatment must be applied or a solution treatment with subsequent age-hardening without exceeding the hardness maximum of the alloy.

From these results, it can be seen that the investigated alloys show after the treatment according to the invention considerably higher properties, particularly for the sealing surface hardness, as compared with their original properties, and that they endure at the same time higher alternating thermal stressings. The Examples show that the Brinell hardness properties after a stabilizing annealing are low.

In view of these results it is shown that cylinder heads treated according to the invention, even those with a higher Mn-content have a considerably longer durability and that the sealing surface hardness is increased. The cylinder heads from such alloys, listed in the following Examples, particularly Cu-containing alloys, show that the alternating load numbers are considerably increased by the application of the thermal treatment of the invention. This important improvement was not to be foreseen at the present state of the art.

Table 10

Strength properties of permanent mold (gravity die) test bars according to the German Air Standard LN 29 531 with a diameter of 22 mm from the manganese-containing Al-Mg-Si alloy without and with copper

| Works<br>Alloy<br>Designation | Average values from two test bars each<br>Composition in % |       |     |      |      |      |      | Heat treatment<br>and quench           | Mechanical Properties |            |            |      |
|-------------------------------|------------------------------------------------------------|-------|-----|------|------|------|------|----------------------------------------|-----------------------|------------|------------|------|
|                               | Cu                                                         | Be    | Mg  | Si   | Mn   | Fe   | Ti   |                                        | $\sigma_{0.2}$        | $\sigma_B$ | $\delta_s$ | HB   |
| 411/1                         | 0.02                                                       | 0.004 | 3.9 | 0.9  | 0.85 | 0.20 | 0.16 | Stabilizing annealing/air              | 10.1                  | 22.9       | 10.6       | 66.5 |
|                               |                                                            |       |     |      |      |      |      | 12 <sup>h</sup> 565°C/H <sub>2</sub> O | 10.5                  | 25.1       | 19.6       | 68.5 |
|                               |                                                            |       |     |      |      |      |      | 12 <sup>h</sup> 565°C/H <sub>2</sub> O | 17.8                  | 29.4       | 15.8       | 85   |
|                               |                                                            |       |     |      |      |      |      | +6 <sup>h</sup> 155°C                  | 19.4                  | 29.5       | 14.1       | 83   |
|                               |                                                            |       |     |      |      |      |      | 12 <sup>h</sup> 565°C/H <sub>2</sub> O | 25.5                  | 33.3       | 6.2        | 110  |
| 411/1<br>+ Cu                 | 0.84                                                       | 0.005 | 4.0 | 0.89 | 0.85 | 0.20 | 0.16 | Stabilizing annealing/air              | 11.4                  | 21.0       | 3.8        | 72.5 |
|                               |                                                            |       |     |      |      |      |      | 12 <sup>h</sup> 565°C/H <sub>2</sub> O | 12.9                  | 28.9       | 12.6       | 75   |
|                               |                                                            |       |     |      |      |      |      | 12 <sup>h</sup> 565°C/H <sub>2</sub> O | 25.5                  | 36.7       | 8.6        | 103  |
|                               |                                                            |       |     |      |      |      |      | +6 <sup>h</sup> 155°C                  |                       |            |            |      |
|                               |                                                            |       |     |      |      |      |      | +6 <sup>h</sup> 175°C                  |                       |            |            |      |

\*) p = ponds

## EXAMPLE 9

Investigations for cylinder heads of an alloy having a composition

|                                                 |                                        |
|-------------------------------------------------|----------------------------------------|
| 0.9                                             | % Mn                                   |
| 3.9                                             | % Mg                                   |
| 0.9                                             | % Si                                   |
| —                                               | % Cu                                   |
| 0.18                                            | % Ti                                   |
| 0.24                                            | % Fe                                   |
| 0.004                                           | % Be                                   |
| Balance                                         | Al                                     |
| Heat treatment and quench                       |                                        |
| 12 <sup>h</sup> 565°C/H <sub>2</sub> O          |                                        |
| + 6 <sup>h</sup> 155°C                          |                                        |
| Alternating load number                         | 1418                                   |
| HB kpounds/mm <sup>2</sup>                      | 80                                     |
| Properties from the border of the cylinder head | $\sigma_{0.2}$ 13.0 kp/mm <sup>2</sup> |
| spherical cap                                   | $\sigma_B$ 27.0 kp/mm <sup>2</sup>     |
|                                                 | 85 10.0 %                              |
|                                                 | 80 kp/mm <sup>2</sup>                  |
| * p = ponds                                     | 8.8 %                                  |

The Brinell hardnesses of cylinder heads made from this alloy were between 60 and 70 kilopounds/mm<sup>2</sup> after stabilizing annealing.

## EXAMPLE 10

Investigations of cylinder heads made of an alloy with

|                                                                      |                                        |
|----------------------------------------------------------------------|----------------------------------------|
| 0.9                                                                  | % Mn                                   |
| 3.9                                                                  | % Mg                                   |
| 0.9                                                                  | % Si                                   |
| 0.8                                                                  | % Cu                                   |
| 0.18                                                                 | % Ti                                   |
| 0.32                                                                 | % Fe                                   |
| 0.004                                                                | % Be                                   |
| Balance                                                              | Al                                     |
| Heat Treatment                                                       |                                        |
| Stabilizing Annealing                                                |                                        |
| 12 <sup>h</sup> 565°C/H <sub>2</sub> O                               |                                        |
| + 6 <sup>h</sup> 175°C                                               |                                        |
| Alternating load number                                              | 1275                                   |
| HB kp/mm <sup>2</sup>                                                | 71                                     |
| Properties from the border of the spherical cap of the cylinder head | $\sigma_{0.2}$ 12.0 kp/mm <sup>2</sup> |
|                                                                      | $\sigma_B$ 18.4 kp/mm <sup>2</sup>     |
|                                                                      | 85 2.9 %                               |
|                                                                      | 71 kp/mm <sup>2</sup>                  |
|                                                                      | 16.8 kp/mm <sup>2</sup>                |
|                                                                      | 32.6 kp/mm <sup>2</sup>                |
|                                                                      | 5.4 %                                  |
|                                                                      | 110 kp/mm <sup>2</sup>                 |
|                                                                      | 27.8 kp/mm <sup>2</sup>                |
|                                                                      | 33.5 kp/mm <sup>2</sup>                |
|                                                                      | 6.6 %                                  |
|                                                                      | 108 kp/mm <sup>2</sup>                 |

\*) p = ponds

## 25

## EXAMPLE 11

With the following alloy in identical cylinder heads according to Examples 9 and 10, the following results were obtained.

|    |                         |      |                                        |
|----|-------------------------|------|----------------------------------------|
| 30 | 0.9                     | % Mn |                                        |
|    | 4.5                     | % Mg |                                        |
|    | 1.5                     | % Si |                                        |
|    | 1.5                     | % Ni |                                        |
|    | 0.2                     | % Cu |                                        |
|    | 0.18                    | % Ti |                                        |
|    | 0.25                    | % Fe |                                        |
|    | 0.004                   | % Be |                                        |
|    | Balance                 | Al.  |                                        |
| 40 | Heat Treatment          |      | 12 <sup>h</sup> 565°C/H <sub>2</sub> O |
|    | Stabilizing Annealing   |      | + 6 <sup>h</sup> 175°C                 |
| 45 | Alternating load number | 1642 | 1700                                   |
|    | HB kp/mm <sup>2</sup>   | 74   | 93                                     |
|    |                         |      | 102                                    |

\*) p = ponds

## 50

## EXAMPLE 12

Further investigations of cylinder heads made of the following alloy gave the following results:

|                         |                       |                                        |  |  |  |  |  |  |  |  |  |
|-------------------------|-----------------------|----------------------------------------|--|--|--|--|--|--|--|--|--|
| 0.9                     | % Mn                  |                                        |  |  |  |  |  |  |  |  |  |
| 5.5                     | % Mg                  |                                        |  |  |  |  |  |  |  |  |  |
| 1.5                     | % Ni                  |                                        |  |  |  |  |  |  |  |  |  |
| 1.5                     | % Si                  |                                        |  |  |  |  |  |  |  |  |  |
| 0.2                     | % Cu                  |                                        |  |  |  |  |  |  |  |  |  |
| 0.18                    | % Ti                  |                                        |  |  |  |  |  |  |  |  |  |
| 0.004                   | % Be                  |                                        |  |  |  |  |  |  |  |  |  |
| Balance                 | Al.                   |                                        |  |  |  |  |  |  |  |  |  |
| Heat Treatment          | Stabilizing Annealing | 12 <sup>o</sup> 565°C/H <sub>2</sub> O |  |  |  |  |  |  |  |  |  |
| Alternating load number | 1091                  | 2184                                   |  |  |  |  |  |  |  |  |  |
| HB kp*/mm <sup>2</sup>  | 85                    | 96                                     |  |  |  |  |  |  |  |  |  |

\* p = ponds

The results of the Examples 9 – 12 reflect the essence of the invention in two respects; firstly, the established thermal treatment removes the influence of unfavorable higher magnesium contents; secondly, after the solution treatment, without disadvantage to the ability to endure alternating thermal stressing, the hardness properties can, even with an increase of the Mg concentration, be increased considerably, without thereby reducing the resistance against alternating thermal stressing of the cylinder heads.

As shown by Examples 9 – 12, a solution heat treatment alone can be sufficient, while a subsequent aging can lead to the obtaining of other desired properties.

- such components further materials with particularly fine structures. This task is accomplished by the invention in such a way that in an Al-Mg-Si alloy, for the indicated purpose, cobalt or chromium or a combination of the two elements act as elements for reducing the solubility of hydrogen to replace completely or partly the manganese content of 0.6 to 2.0% indicated for other alloys of the invention. The replacement is to be on the basis of equivalent numbers of gram-atoms. 5 Preferably at least 0.1% Co and/or at least 0.6% Cr is present. In this manner, a grain refining of the structure of components is attained which lends to these components additional outstanding properties. Thus, there can be found in the structure in the case of chromium 10 larger islands with very fine Mg<sub>2</sub>Si. Moreover, the resistance of components, e.g. of cylinder heads, made of Al-Mg-Si alloys, which contain within the indicated limits besides manganese partly cobalt and/or chromium, is excellent. 15 Also vanadium and molybdenum can be used as elements for reducing the solubility of hydrogen. They replace the manganese content on the basis of equivalent numbers of gram-atoms. At least 0.1% V and/or at least 0.1% Mo is preferably present in such alloys. 20 Table 11 shows the effect of Cr, Co, V, and Mo in alloys of the invention. Charge Nos. 850 and 2606 are presented for purposes of comparison. 25

TABLE 11  
Strength values determined using chill-mold rod castings according to German Aviation Standard (Luftfahrtnorm) LN 29531 with 22 m diam; average of three values; influence of Cr, Co, V, and Mo.

| Works Alloy No. or Charge No. | Analysis in % |                |            |                           |              |              | Heat Treatment | Mechanical Values                                  |                                   |              |                           |          |
|-------------------------------|---------------|----------------|------------|---------------------------|--------------|--------------|----------------|----------------------------------------------------|-----------------------------------|--------------|---------------------------|----------|
|                               | Cu            | Be             | Mg         | Si                        | Mn           | Fe           | Ti             | $\sigma_{0.2}$<br>kp*/mm <sup>2</sup>              | $\sigma_B$<br>kp*/mm <sup>2</sup> | $\delta_s\%$ | HB<br>kp*/mm <sup>2</sup> |          |
| 850<br>(s. Tab.2)<br>2612     | —<br>0.005    | n.b.<br>0.0035 | 3.6<br>3.5 | 1.04<br>0.95<br>+ 0.6% Cr | 0.22<br>0.01 | 0.31<br>0.22 | n.b.<br>0.19   | Stabilizing Annealing<br>do.                       | 7.7<br>10.3                       | 17.1<br>21.8 | 6.1<br>9.4                | 54<br>64 |
| 2613                          | 0.005         | 0.0045         | 3.6        | 0.92<br>+ 0.1% Co         | 0.01         | 0.23         | 0.21           | do.                                                | 8.3                               | 20.7         | 14.1                      | 60       |
| 2614                          | 0.01          | 0.004          | 3.65       | 0.94<br>+ 0.6% Co.        | 0.01         | 0.27         | 0.22           | do.                                                | 8.5                               | 21.9         | 15.6                      | 62       |
| 2615                          | 0.005         | 0.004          | 3.55       | 0.91<br>+ 0.1% V          | 0.01         | 0.20         | 0.21           | do.                                                | 8.2                               | 19.4         | 8.0                       | 59       |
| 2684                          | 0.015         | 0.0045         | 3.7        | 0.85<br>+ 0.6% Mo         | 0.02         | 0.23         | 0.19           | do.                                                | 8.7                               | 19.6         | 7.9                       | 63       |
| 2606                          | 0.90          | 0.003          | 4.4        | —<br>1.52                 | 0.01         | 0.17         | 0.22           | Solution Heat Treatment +<br>6 hrs at 175°C<br>do. | 19.7                              | 28.8         | 6.2                       | 97       |
| 2613                          | 0.85          | 0.004          | 4.5        | —<br>1.55                 | 0.01         | 0.21         | 0.19           | do.                                                | 18.3                              | 28.9         | 8.0                       | 98       |
|                               | 0.88          | 0.005          | 4.7        | 1.45<br>+ 0.6% Co         | 0.01         | 0.23         | 0.19           | do.                                                | 20.1                              | 31.5         | 8.5                       | 102      |
| 2615                          | 0.88          | 0.0045         | 4.5        | 0.51<br>+ 0.1% V          | 0.01         | 0.17         | 0.19           | do.                                                | 18.1                              | 29.6         | 10.0                      | 94       |
| 2683                          | 0.86          | 0.004          | 4.7        | 1.57<br>+ 0.1% Mo         | 0.02         | 0.25         | 0.20           | do.                                                | 20.5                              | 30.7         | 8.3                       | 101      |

Thus, in Example 12 where there is a high free Mg content, a solution heat treatment alone can give very respectable properties. In contrast, Examples 9 – 11 show that, for a lower free Mg content, an aging in addition to the solution treatment can be of advantage. Then, it remains to be noted that, when a very high Brinell hardness is required for sealing surfaces, for example for surface 18 in FIG. 3, an age hardening can be of advantage as shown, for example, in Example 11.

The present invention also leads to the further development of alloys for components which are subjected to maximum alternating thermal stresses, particularly for cylinder heads for combustion engines, the materials for which are based on the Al-Mg-Si alloys of the invention. This further development aimed at finding for

55 It is preferred to use technically pure aluminum. Percentages herein are in percent by weight unless indicated otherwise.

It will be understood that the above description of the present invention is susceptible to various modifications, changes and adaptations, and the same are intended to be comprehended within the meaning and 60 range of equivalents of the appended claims.

I claim:

1. A high-strength manganese-containing Al-Mg-Si alloy having a free magnesium content of 1.5 to 4%, said alloy consisting essentially of 0.6 to 1.8% manganese, 2 to 7% magnesium, 0.6 to 2.5% silicon, 0.1 to 0.3% titanium, and having been subjected to one of the 65 following steps (a) and (b):

- a. a solution treatment up to 565° C maximum;
- b. a corresponding solution treatment with subsequent age-hardening at temperatures not exceeding the hardness maximum.
- 2. An alloy as claimed in claim 1, said alloy containing up to 1.5% Ni, up to 3% Cu, up to 0.1% beryllium, and at most 0.6% Fe.
- 3. An alloy as claimed in claim 1, said alloy containing manganese only in the quantities up to 1.2%, magnesium from 3.0 to 4.5%, silicon from 0.8 to 1.2%, and copper from 0.2 to 1.0%.
- 4. An alloy as claimed in claim 1, the magnesium content of said alloy being from 4.5 to 7.5% and the silicon content of said alloy being 0.8 to 2.5%.
- 5. An aluminum-magnesium-silicon alloy consisting essentially of 0.6 to 4.5% silicon, 2.5 to 11% magnesium, and aluminum, wherein the improvement comprises 1 to 4.5% free magnesium and at least one mate-

- rial selected from the group consisting of manganese at 0.6 to 1.8%, cobalt, chromium, vanadium, and molybdenum, where the sum of the gram-atoms of manganese, cobalt, vanadium, and molybdenum lies in the gram-atom range equivalent to 0.6 to 1.8% manganese.
- 6. An alloy as claimed in claim 5, said alloy containing at least one element selected from the group consisting of cobalt at at least 0.1% and chromium at at least 0.6%.
- 7. An alloy as claimed in claim 5, said alloy containing up to 1.5% Ni, up to 0.5% Cu, and at most 0.6% Fe.
- 8. An alloy as claimed in claim 5, said alloy containing 3% free magnesium.
- 9. An alloy as claimed in claim 5, said alloy containing at least one element selected from the group consisting of vanadium at at least 0.1% and molybdenum at at least 0.1%.

\* \* \* \* \*

UNITED STATES PATENT OFFICE  
CERTIFICATE OF CORRECTION

Patent No. 3,868,250

Dated February 25, 1975

Inventor(s) Paul Zimmermann

It is certified that error appears in the above-identified patent and that said Letters Patent are hereby corrected as shown below:

Columns 9, 10, 11 and 12 as shown on the attached pages should be added:

**Signed and Sealed this**  
*sixteenth Day of September 1975*

[SEAL]

*Attest:*

**RUTH C. MASON**  
*Attesting Officer*

**C. MARSHALL DANN**  
*Commissioner of Patents and Trademarks*

## BRIEF DESCRIPTION OF THE DRAWINGS

FIG. 1 is a graph of alternating load number versus the percentage of free magnesium in an alloy.

FIG. 2 is a graph of the percentage of silicon in an alloy versus the percentage of magnesium and shows the field of free magnesium contents between 1 and 3%.

FIG. 3 is a cross section through a portion of an air-cooled cylinder head according to the invention.

## DESCRIPTION OF THE PREFERRED EMBODIMENTS

Preferred elements for reducing the solubility of hydrogen in the melt above 700° C are manganese and nickel.

The available results were applied to investigations of cylinder heads. The quality of service to be expected from an alloy used to make a cylinder head was measured in terms of "alternating load number," which is measured as follows.

On a heatable and coolable test stand, those portions of a cylinder head as are most endangered, being nearest to the combustion chamber, are heated for approximately 60 seconds from a temperature of 100° to 300° C and then cooled in 60 seconds to 100° C again. This effects a change of load. The test on the test stand is carried on until crack formation and then on until the crack has progressed through the wall where it is located. The number of load changes supported by the cylinder head until crack formation and until crack-through yields alternating load numbers, which serve as an indicator of the ability to resist thermal fatigue.

FIG. 1 shows among other things the alternating thermal stress tests of cylinder heads made of the customary alloy AlMg5SiCu0.5 per Table 7. The cylinder heads of Table 7 were taken from the normal production in a period extending over several months. There resulted an average alternating load number of 716 until crack formation and 769 until crack-through.

Cylinder heads cast from the material of the inven-

tion and showing a fine grain structure were likewise tested. FIG. 1 and Table 8 show the resulting alternating load numbers. It can be concluded from the investigations that with a silicon content comparable with the customary alloy, and with the customary addition of 0.5% Cu, alloys with high magnesium contents have a considerably shorter operating life even with an additional manganese-alloying. In comparison with the results for the customary alloy (see FIG. 1 and Tables 7 and 8), the alloys with higher manganese content show a distinct improvement. The graph in FIG. 1 shows an almost linear dependence between alternating load number and magnesium content and the possibility of a maximum improvement of 100% by the invention. The alloy used for cylinder head No. 3 in Table 8 and FIG. 1 possesses a free (i.e., not present in Mg<sub>2</sub>Si) magnesium-content of approximately 5.7%; the alloy of head No. 2 has a free magnesium-content of 3.77%, and the alloy of head No. 1 has a free magnesium-contents of only 2.85%. The alloys of heads No. 4 and No. 5 in Table 8 contain only about 0.9% free magnesium. The alloy of head No. 5 endures after the additional alloying of manganese considerably higher thermal loading. Comparison with the alloys of Table 7 shows the high thermal stress endurance obtained by the reduction of the free magnesium content. The free magnesium content of the alloys Nos. 4 and 5, being 0.9%, is very low. The machinability of these alloys was worse on a production line. The free magnesium contents should be more than 1%.

The alloys of the invention can also be used as wrought material, if the Si-content is at least 1%

All investigations show that the free magnesium-contents of the aluminum-magnesium-silicon alloys for obtaining high endurance, specially against alternating thermal stresses, should be between 1 and 4.5, preferably at 3.0%, a decrease of free magnesium to less than 1% being possible only for castings that are machined with special tools adapted to the alloy. In the presence of more than 0.6% Mn the preferred 3% free magnesium can go up to about 4.5%.

Table 7

| Cylinder Head No. | Analysis in % |      |      |      |      | Alternating load No. |               |
|-------------------|---------------|------|------|------|------|----------------------|---------------|
|                   | Mg            | Si   | Mn   | Cu   | Fe   | Crack formation      | Crack-through |
| 1                 | 5.06          | 0.94 | 0.36 | 0.53 | 0.45 | n.b.                 | 709           |
| 2                 |               |      |      |      |      | 639                  | 670           |
| 3                 |               |      |      |      |      | 894                  | 960           |
| 4                 |               |      |      |      |      | 940                  | 1050          |
| 5                 | 5.19          | 0.99 | 0.36 | 0.52 | 0.44 | 450                  | 640           |
| 6                 |               |      |      |      |      | 775                  | 877           |
| 7                 |               |      |      |      |      | 707                  | 872           |
| 8                 |               |      |      |      |      | 574                  | 736           |
| 9                 |               |      |      |      |      | 640                  | 661           |
| 10                |               |      |      |      |      | n.b.                 | 760           |
| 11                |               |      |      |      |      | 830                  | 880           |
| 12                |               |      |      |      |      | n.b.                 | 650           |
| 13                | 5.16          | 0.95 | 0.36 | 0.55 | 0.43 | n.b.                 | 720           |
| 14                |               |      |      |      |      | n.b.                 | 660           |
| 15                |               |      |      |      |      | n.b.                 | 671           |
| 16                |               |      |      |      |      | n.b.                 | 800           |
| Average values    | 5.14          | 0.96 | 0.36 | 0.54 | 0.44 | 716                  | 769           |

n.b. = not precisely determinable

Table 8

| Cylinder Head No | Analysis in % |      |      |      |      |      |       | Alternating load     |                      |
|------------------|---------------|------|------|------|------|------|-------|----------------------|----------------------|
|                  | Mg            | Si   | Mn   | Cu   | Fe   | Ti   | Be    | No Crack formation   | Crack-through        |
| 1                | 4.55          | 0.99 | 0.91 | 0.50 | 0.42 | 0.15 | 0.004 | 1450<br>1350         | 1600<br>1500         |
| 2                | 5.5           | 1.00 | 0.92 | 0.50 | 0.32 | 0.15 | 0.004 | 890<br>1200          | 890<br>1224          |
| 3                | 7.4           | 0.98 | 0.89 | 0.55 | 0.33 | 0.15 | 0.003 | n.b.<br>n.b.         | 168<br>335           |
| 4                | 4.4           | 2.08 | 0.02 | 0.17 | 0.20 | 0.15 | 0.004 | 1040<br>930<br>n.b.  | 1160<br>1030<br>1100 |
| 5                | 4.3           | 1.88 | 0.78 | 0.15 | 0.21 | 0.15 | 0.004 | 1380<br>1380<br>1360 | 1590<br>1420<br>1410 |

n.b. = not precisely determinable

During the further development of the alloys of the invention and of their applicability, it has been established by thermal alternating stress investigations that, within the range of the limits of the invention, alloys with the following alloying constituents have particularly favorable properties for enduring high-temperature alternating stresses and a particularly low cracking-tendency in engine operation:

|                                          |    |
|------------------------------------------|----|
| 3.5 - 7.0%                               | Mg |
| 0.8 - 2.5%                               | Si |
| 0.6 - 1.5%                               | Mn |
| 0.0 - 0.30%                              | Ti |
| 0.0 - 0.005%                             | Be |
| 0.0 - 0.05% other elements individually. |    |
| total however 0.15% maximum              |    |

Balance aluminum and customary contaminants, on the condition that only 1 to 3% magnesium unbound to silicon be contained in the alloy. A special importance is, in this instance, attributed to the proportioning of the manganese on which the increase of crack resistance in engine operation depends.

The proposed alloy selection results in particularly favorable mechanical properties. But all alloys, both those named first, and those selected now, yield especially improved mechanical properties and to the present time, the best crack resistance against temperature changes, if the endangered or highly stressed areas of the cast body are subjected during the solidification to a cooling additional to the cooling received by other areas of the body. The behavior of alloys free of manganese shows in cylinder heads 30 to 50% of the durability achieved in cylinder heads made of alloys containing manganese.

FIG. 2 shows the range of preferred alloy compositions wherein only 1 to 3% free magnesium (not bound to silicon) is present.

Further illustrative of the invention are the following Examples:

#### EXAMPLE 1

Cylinder heads of the type illustrated by air-cooled

cylinder head 10 in FIG. 3 from an alloy poor in manganese, having the composition

|           |
|-----------|
| 0.3% Mn   |
| 5.2% Mg   |
| 1.0% Si   |
| 0.004% Be |

balance Al and customary contaminants, were subjected to an alternating thermal stress investigation after cooling the permanent mold with about 700 cm<sup>3</sup> H<sub>2</sub>O in the area of the spherical cap 11. The cooling was carried out by flowing the water through a metal mold core abutting against the spherical cap 11 and having cylinder inserts protruding into the inlet channel 12 and the outlet channel 13. The cooling effect provided by the cylinder inserts provides an additionally improved microstructure in the web 14, which is the most highly stressed portion of the head. The alternating load number was approximately 450 for the start of cracking of the web area between the inlet and outlet channels. Additionally in FIG. 3, axes 15, 16 and 17 are axes of cylindrical symmetry for, respectively, the inlet channel 12, the spherical cap 11, and the outlet channel 13.

#### EXAMPLE 2

50 Cylinder heads of the same alloy as in Example 1 showed, after being cooled with 3.5 liters H<sub>2</sub>O in the same area, an alternating load number of 750.

#### EXAMPLE 3

55 Cylinder heads of the manganese rich alloy with the composition

|           |
|-----------|
| 0.9% Mn   |
| 4.4% Mg   |
| 1.0% Si   |
| 0.004% Be |

balance Al and customary contaminants, were subjected, after cooling as in Example 2, to an alternating thermal stress test and yielded an alternating load number of 1,550 to crackthrough.